

July 14, 1953

J. WHARTON ET AL

2,645,555

MANUFACTURE AND PRODUCTION OF ARTIFICIAL THREADS FROM VISCOSE

Filed Jan. 27, 1949

2 Sheets-Sheet 1



Inventors

John Wharton

Ronald Bertram Hall

By their attorneys

Howson and Howson

July 14, 1953

J. WHARTON ET AL

2,645,555

MANUFACTURE AND PRODUCTION OF ARTIFICIAL THREADS FROM VISCOSE

Filed Jan. 27, 1949

2 Sheets-Sheet 2



FIG.2.

Inventors

John Wharton

Ronald Bertram Hall

By their attorneys

Howson and Howson

## UNITED STATES PATENT OFFICE

2,645,555

## MANUFACTURE AND PRODUCTION OF ARTIFICIAL THREADS FROM VISCOSE

John Wharton and Ronald Bertram Hall, Coventry, England, assignors to Courtaulds Limited, London, England, a British company

Application January 27, 1949, Serial No. 73,136  
In Great Britain February 18, 1948

11 Claims. (Cl. 18—54)

1

This invention relates to the manufacture and the production of artificial threads, filaments, yarns and the like, hereinafter referred to as threads, from viscose.

In the production of artificial threads from viscose, viscose is extruded through a jet into a coagulating bath containing sulphuric acid and one or more metallic salts. The threads are withdrawn from the coagulating bath and passed by means of thread guides over one or more godets, or the threads are passed on to one or more thread-advancing reels where they are treated with processing liquids. Insoluble substances are formed by the reaction which takes place during the coagulation and subsequent treatment of the thread and these substances are carried away by the thread and tend to form hard deposits on thread guides, godets and thread-advancing reels.

It has already been proposed in U. S. Letters Patent specification No. 2,125,031 to add to the spinning bath or to the spinning solution an organic substance the molecule of which has a surface-active cation derived from an organic base substituted by an aliphatic chain of high molecular weight in order to inhibit the fouling of the jets. It has also been proposed in the specification of U. S. Letters Patent No. 2,394,519 to extrude viscose into an acidic coagulating liquid containing an emulsified petroleum oil, which is insoluble in the liquid and forms a sludge with impurities in the coagulating liquid and tends to inhibit the formation of harmful deposits not only in and upon the jets but also upon other parts of the apparatus.

The object of the present invention is to improve the production of artificial threads from viscose by preventing the formation of rock-like deposits and inerustations on thread guides, godets or thread-advancing reels and to effect lubrication of the thread during its manufacture.

The present invention consists of a process for the production of artificial threads from viscose by extruding the viscose into a coagulating bath containing an acid and one or more metallic salts wherein the thread after leaving the coagulating bath is treated with an oil having dissolved in it an oil-soluble cation-active compound.

The treatment with the oil having dissolved in it an oil-soluble cation-active compound is preferably applied to the thread prior to the application of a processing liquid containing sulphuric acid and one or more metallic salts.

The present invention may conveniently be

2

used in a process in which the threads after leaving the coagulating bath are stretched whilst immersed in a bath of hot dilute acid, for example, as described in U. S. Letters Patent specification No. 2,192,074. With such processes the treatment with the oil having dissolved in it the oil-soluble cation-active compound is preferably applied before the thread passes into the bath of hot dilute acid.

10 When carrying out the process of the present invention the oil having dissolved in it the oil-soluble cation-active compound is preferably allowed to drip on to the thread while it is passing over a godet or a thread-advancing reel.

15 In practice for economic reasons and for general usefulness the oil employed is a mineral oil such as that known as "white oil," the term "oil" is used in this specification to cover any organic liquid which may be used for the lubrication of

20 solid surfaces, for example, vegetable oils, such as olive oil or cotton seed oil and animal oils such as sperm oil. It is desirable that the cation-active compound should be soluble in the oil being employed to such an extent that a clear

25 solution is obtained, but total solubility is not essential provided the oil and cation-active compound may be delivered to the machine without separation. It will therefore be necessary to select a cation-active compound according to the oil being used. The following classes of cation-active compounds will normally be found sufficiently soluble in the mineral oil which will be commonly used in practice.

30 1. Condensation products of the general formula  $R.CO.(NHC_2H_4)_n-NH_2$  in which R is a long chain hydrophobe group with not less than 10 carbon atoms in the chain and n is an integer of 1 to 5. These compounds are obtained by condensing a long chain fatty acid with an aliphatic polyamine, for example by condensing 1 mol of oleic, stearic or palmitic acid or a mixture of these acids with 1 mol of diethylene triamine, triethylene tetramine or pentaethylene hexamine or a mixture of these polyamines, at about 180° centigrade for three hours.

35 2. Condensation products of the general formula:



40 in which R is a long chain hydrophobe group with not less than 10 carbon atoms in the chain, n is an integer of 1 to 5, R', R'' are alkyl groups, for example methyl or ethyl groups, and X is an

anion for example  $\text{Br}^-$ ,  $\text{HSO}_4^-$  or  $\text{CH}_3\text{COO}^-$ . These condensation products may be obtained by alkylating the condensation products from long chain fatty acids and aliphatic polyamines as described in class 1 by treatment for example with dimethyl or diethyl sulphate at about 16° centigrade.

3. Condensation products obtained by reacting a long chain fatty acid, having not less than 10 carbon atoms in the chain for example oleic acid or stearic acid, with an alkanolamine, for example mono-ethanolamine, and also the products obtained by reacting such condensation products with an alkylene oxide, for example ethylene oxide providing that the ethylene oxide is restricted so that the oil-soluble properties are retained.

4. Condensation products obtained by reacting a long chain aliphatic primary amine, for example octadecylamine, with an alkylene oxide, for example ethylene oxide, until a product is formed which is just dispersible in water.

5. Condensation products obtained by reacting a long chain aliphatic primary amine with ethylene oxide and alkylating the product obtained by treatment, for example, with dimethyl or diethyl sulphate. The general formula of the condensation products obtained is:



in which R is a long chain hydrophobe group with not less than 10 carbon atoms, R' and R'' are alkyl groups, X is an anion, for example  $\text{Br}^-$ ,  $\text{HSO}_4^-$  or  $\text{CH}_3\text{COO}^-$ , and n is an integer of 2 to 20 according to the chain length of R.

The most effective oil-soluble cation-active compounds for carrying out the present invention are those which will form emulsions when the oil containing the cation-active compound is shaken up with dilute aqueous solutions containing sulphuric acid and one or more metallic salts.

In the production of artificial threads from viscose of high denier, for example a thread of 1180 denier 500 filament, the formation of rock-like deposits on those parts of the spinning machine with which the threads come into contact immediately after leaving the coagulating bath is particularly rapid so that treatment of the thread on the first godet or thread-advancing device with oil having dissolved in it an oil-soluble cation-active compound in accordance with the present invention is of particular value.

The process of the present invention is particularly useful in the continuous spinning process in which the thread is withdrawn from the coagulating bath and passed over one or more thread-advancing reels in a number of helical turns, the thread being treated with processing liquids during its passage over the reels. By dripping oil having dissolved in it an oil-soluble cation-active compound on to the thread at the delivery end of the first-thread-advancing reel in accordance with the present invention the thread takes up the oil and retains it in sufficient quantity to lubricate the thread during its passage and treatment on subsequent reels. The sulphur impurities remain soft and are carried away by the movement of the thread and the processing liquids. The thread-advancing reels remain substantially free from rock-like deposits which would have a deleterious action on the thread as well as necessitating frequent and arduous cleaning operations.

The accompanying diagrammatic drawings further illustrate the process of the present invention:

5 Figure 1 represents part of a continuous spinning machine and,

Figure 2 represents part of a centrifugal spinning machine.

Referring to Figure 1, viscose is extruded from the jet 1 from the supply pipe 2 into the coagulating bath 3 to form the thread 4. The coagulating bath 3 may conveniently contain sulphuric acid and one or more metallic salts. The thread 4 leaving the coagulating bath 3 passes upwards to the thread-advancing device 5 over which it travels in a number of advancing helical turns. Oil having dissolved in it an oil-soluble cation-active compound is allowed to drip on to the thread 4 from the distributor 6 while the thread is passing over the thread-advancing device 5. On reaching the discharge end of thread-advancing device 5 the thread passes vertically downwards to thread-advancing device 7 and thence to thread-advancing devices 8, 9 and 10, over each of which it travels in a number of advancing helical turns. While the thread is travelling over thread-advancing devices 7, 8 and 9 it may be subjected to treatment with one or more processing liquids for example, washing, desulphurising and bleaching liquids, the processing liquids being supplied by the distributors 11, 13 and 15 and the used processing liquids being collected in drip pans 12, 14 and 16. The thread-advancing device is supplied internally with steam for heating and drying the thread. The dried thread is collected on a holder 17 by the cap spinning device 18. The dripping of oil having dissolved in it an oil-soluble cation-active compound onto the thread travelling on thread-advancing device 5 prevents the formation of rock-like deposits on thread-advancing devices 5, 7, 8, 9 and 10, so that the machine can be operated for long periods without stoppages for cleaning.

Referring to Figure 2, viscose is extruded from the jet 20 from the supply pipe 21 into the coagulating bath 22 to form the thread 23. The coagulating bath may conveniently contain sulphuric acid and one or more metallic salts. The thread 23 leaving the coagulating bath 22 passes on to the godet 25 by means of thread-guide 24. Oil having dissolved in it an oil-soluble cation-active compound is allowed to drip from the distributor 26 onto the thread passing over the godet 25. The thread leaving godet 25 passes up to godet 27 and is then guided by the spinning funnel 28 into the rapidly rotating box 29 where the thread is collected in the form of a cake. The godets 25, 27, thread-guide 24 and spinning funnel 28 remain free from rock-like deposits.

The addition of less than 10 per cent on the weight of oil of an oil-soluble cation-active compound according to the process of the present invention gives the thread an affinity for the oil so that the oil is retained on the thread in sufficient quantity to lubricate the thread during subsequent treatment. The oil retained on the thread may be sufficient to render the usual soaping or finishing treatment unnecessary.

The present invention therefore prevents the formation or rock-like deposits on thread guides, godets and thread-advancing reels and effects lubrication of the thread while economising in the quantity of oil used.

The following examples illustrate the present

invention, the percentages and parts being by weight:

*Example 1*

Viscose is extruded through a multi-hole jet into a coagulating bath containing 10 per cent of sulphuric acid, 18 per cent of sodium sulphate and 1 per cent of zinc sulphate. The thread is withdrawn from the coagulating bath and passed onto the delivery end of a thread-advancing reel where it is immediately treated by dripping on it at the rate of 0.25 cm.<sup>3</sup> per minute a 5 per cent solution in mineral oil of a cation-active compound obtained by condensing 1 mol of oleic acid with 1 mol of triethylene tetramine at 180° centigrade for 3 hours. The thread is then sprayed with a solution containing 1.5 per cent of sulphuric acid, 5 per cent of sodium sulphate and 0.2 per cent of zinc sulphate. The thread reaches the discharge end of the reel and then passes on to a second thread-advancing reel. The thread has retained sufficient oil to lubricate the second reel and to prevent formation of hard deposits on both reels.

*Example 2*

Viscose thread leaving the coagulating bath is passed on to a thread-advancing reel where it is sprayed at the rate of 0.2 cm.<sup>3</sup> per minute with a 5 per cent solution in olive oil of a cation-active compound obtained by alkylating at room temperature with 1 mol of dimethyl sulphate the condensation product of 1 mol of palm kernel oil with 1 mol of diethylene triamine. The thread is then sprayed with a solution containing 2 per cent of sulphuric acid, 4.2 per cent of sodium sulphate and 0.5 per cent of zinc sulphate. The treatment with the oil containing the cation-active compound prevents harmful deposits of sulphur impurities forming on the reel since the oil retained by the thread lubricates the reel. The thread obtained after washing is soft and pliable and does not require soaping.

*Example 3*

Viscose rayon thread of 1180 denier, 500 filaments is withdrawn from the coagulating bath and passed round a godet. A 3 per cent solution in mineral oil of a cation-active compound obtained by condensing 1 part of stearyl ethanolamide with 2 parts of ethylene oxide is dripped on to the thread passing over the godet at the rate of 0.2 cm.<sup>3</sup> per minute. The thread is then passed through a hot dilute acid bath containing from 0.5 to 4 per cent of sulphuric acid, from 1 to 12 per cent of sodium sulphate and from 0. to 1.5 per cent of zinc sulphate and subjected to a stretching as described in U. S. Letters Patent specification No. 2,192,074. The thread retains sufficient oil, even after its passage through the stretching bath to prevent deposits on the thread guides and godets over which the thread is passed after leaving the stretching bath.

What we claim is:

1. A process for the production of artificial threads from viscose by extruding viscose into a coagulating bath containing sulphuric acid and at least one metallic sulphate including as the first step after the thread leaves the coagulating bath, a step of treating the thread with a solution consisting of an oil selected from the group consisting of mineral oils, vegetable oils and animal oils and a cation-active compound soluble in the oil.

2. A process as claimed in claim 1 wherein the oil-soluble cation-active compound is a condensation product obtained by condensing a long chain fatty acid with an aliphatic polyamine.
3. A process as claimed in claim 1 wherein the oil-soluble cation-active compound is the condensation product obtained by reacting a long chain fatty acid having not less than 10 carbon atoms in the chain with an alkanolamine.
4. A process as claimed in claim 1 wherein the oil-soluble cation-active compound is the condensation product obtained by reacting a long chain aliphatic primary amine with an alkylene oxide until a water-dispersible product is found.
5. A process as claimed in claim 1 wherein the oil-soluble cation-active compound is oleyl polyamide obtained by condensing oleic acid with triethylene tetramine.
6. A process as claimed in claim 1 wherein the oil-soluble cation-active compound is oleyl ethanolamide.
7. A process for the production of artificial threads from viscose by extruding viscose into a coagulating bath containing sulphuric acid and at least one metallic sulphate, including as the first step after the thread leaves the coagulating bath, a step of treating the thread with a solution consisting of mineral oil and a cation-active compound soluble in the oil.
8. A continuous process for the production of artificial threads from viscose by extruding viscose into a coagulating bath containing sulphuric acid and at least one metallic sulphate and subjecting the thread thus formed without any break to a series of treatment liquids and to drying and winding onto a package, including as the first step after the thread leaves the coagulating bath, a step of treating the thread with a solution consisting of an oil selected from the group consisting of mineral oils, vegetable oils and animal oils and a cation-active compound soluble in the oil.
9. A continuous process for the production of artificial threads from viscose by extruding viscose into a coagulating bath containing sulphuric acid and at least one metallic sulphate and subjecting the thread thus formed without any break to a series of treatment liquids and to drying and winding onto a package, including as the first step after the thread leaves the coagulating bath, a step of treating the thread with a solution consisting of mineral oil and a cation-active compound soluble in the oil.
10. A process for the production of artificial threads from viscose by extruding viscose into an aqueous coagulating bath containing sulphuric acid and at least one metallic sulphate including the step of treating the thread after it leaves the coagulating bath with a solution consisting of an oil selected from the group consisting of mineral oils, vegetable oils and animal oils and a cation-active compound soluble in the oil and treating the thread subsequently with an aqueous processing liquid containing sulphuric acid and at least one metallic sulphate.
11. A process for the production of artificial threads from viscose by extruding viscose into an aqueous coagulating bath containing sulphuric acid and at least one metallic sulphate including the step of treating the thread after it leaves the coagulating bath with a solution consisting of an oil selected from the group consisting of mineral oils, vegetable oils and animal oils and a cation-active compound soluble in the oil and
- 75 a cation-active compound soluble in the oil and

stretching the thread subsequently in a hot dilute acid bath.

JOHN WHARTON.  
RONALD BERTRAM HALL.

References Cited in the file of this patent

UNITED STATES PATENTS

| Number    | Name             | Date          |
|-----------|------------------|---------------|
| 1,970,578 | Schoeller et al. | Aug. 21, 1934 |
| 2,125,031 | Polak et al.     | July 26, 1938 |

Number  
2,214,352  
2,309,072  
2,329,086  
5 2,345,570

| Name             | Date           |
|------------------|----------------|
| Schoeller et al. | Sept. 10, 1940 |
| Burkholder       | Jan. 19, 1943  |
| Robinson et al.  | Sept. 7, 1943  |
| Eley             | Apr. 4, 1944   |

FOREIGN PATENTS

| Number  | Country       | Date          |
|---------|---------------|---------------|
| 546,051 | Great Britain | June 25, 1942 |